# EUROPEAN PATENT SPECIFICATION

(11) **EP 0 369 692 B1**
(45) Date of publication and mention of the grant of the patent: **19.05.1993**
(21) Application number: 89311655.8
(22) Date of filing: 10.11.1989
(51) Int. Cl.: C10M 173/02

(54) **Water based functional fluids**
Wässrige funktionelle Flüssigkeiten
Fluides fonctionnels à base d'eau

(30) Priority: 17.11.1988 GB 8826857
(43) Date of publication of application: 23.05.1990
(73) Proprietor: BP Chemicals Limited, London EC2M 7BA (GB)
(72) Inventor: Faulks, James Neville Gardiner BP Chemicals Ltd., London, SW1W 0SU (GB); Moxey, John Robert Hythe Chemicals limited, Hythe, Southampton Hants, S04 6ZG (GB)
(74) Representative: Barlow, Michael Thomas

(56) References cited:
- GB-A- 1 182 448
- US-A- 4 312 775
- US-A- 4 481 125
- US-A- 4 767 555

## Description

The present invention relates to the use of water based functional fluids which can be used for example as hydraulic fluids, lubricants, drilling or cutting fluids.

Functional fluids based upon mixtures of water and polyether glycols are well known and are used in a wide variety of applications eg as cutting fluids, hydraulic fluids and the like.

Typical formulations of water-based hydraulic fluids (known as HF-C fluids) comprise approximately 15-30% of a high-viscosity polyether glycol, and 35-45% water, with the balance (up to 50%) being simple glycol and small amounts of additives known to the skilled man. Typically these hydraulic fluids have a viscosity of 32-68 cSt at 40°C.

There is a growing trend however to reduce the polyether glycol content of such functional fluids. For example it would ultimately be desirable to reduce the polyether glycol content of hydraulic fluids to 10% or possibly even less. There is also a trend to produce what can be described as High Water Based Fluids (HWBFs), containing typically 50-98 percent water, by additionally removing some or all of the glycol.

A problem arises when attempts are made to reduce the polyether glycol content of hydraulic fluids in that the viscosity of the hydraulic fluid is reduced. This arises because standard polyether glycol fluids do not possess sufficient thickening power. Simply increasing the viscosity of the polymer does not achieve the required effect, because the increase in solution viscosity becomes marginal, and the polymer becomes unstable under conditions of high shear.

It has previously been proposed for example in US 4 767 555 and US 4 288 639 to achieve the required viscosity of such hydraulic fluids by incorporation of small amounts of materials which (a) are water compatible and (b) increase the viscosity of the hydraulic fluids by intermolecular association in solution. Such materials are known as associative thickeners

The hydraulic fluids previously described as high-water-based fluids (HWBFs), usually incorporating either no simple glycol, or only small amounts as antifreeze, have a number of disadvantages when compared to HFC water glycol fluids, viz
i) Although the HWBFs normally exhibit 'permanent shear stability', that is the viscosity of the fluid remains stable over a long period of operation, they none-the-less exhibit temporary loss of viscosity in high shear zones, as evidenced by loss of flow rate and pump efficiency in hydraulic systems, in other words they lack 'temporary shear stability'.
ii) Under such conditions of temporary viscosity loss, hydrodynamic lubricity of the fluid also suffers. Lubrication is maintained only by additives which provide boundary lubrication (EP additives). Despite such additives being highly developed, these conditions can result in enhanced wear. Additionally the best of these additives in many instances are toxic, hydrolytically unstable and environmentally undesirable.
iii) The viscosity index of such fluids is often poor which can give problems with pump start-up.
iv) HWBF's are sensitive to water loss, which has a dramatic and undesirable effect on fluid viscosity.

US 3538033 discloses a family of polyether derivatives of diepoxides which can be used as thickeners in textile printing emulsions, cosmetic emulsions, aqueous pigment suspensions and the like.

GB 1182448 discloses thickening agents for use in textile printing emulsions and cosmetic emulsions. These thickening agents are made by preparing an adduct of at least 20 mols of an alkylene oxide and one mole of a starter such as a monohydric aliphatic alcohol and reacting the adduct with a diepoxide compound.

US 4390440 discloses water or water/glycol based hydraulic fluids containing a thickening agent. However these thickening agents are prepared by reacting a starter molecule, one or more alkylene oxides and a monoepoxide.

The problem to be solved is therefore to produce functional fluids, suitable for the applications described above, which have good permanent and temporary shear stability, contain low concentrations of the associative thickeners, have good resistance to water loss in terms of viscosity change, have good apparent viscosity indices, and which maintain hydrodynamic lubrication under high shear conditions.

According to the present invention there is provided a functional fluid composition for use as a hydraulic fluid, lubricant, a cutting fluid or a drilling fluid which comprises
(a) from 20 to 98% by weight water
(b) a finite amount up to 79.5% by weight of a glycol and
(c) from 0.5 to 25% by weight of a thickening agent prepared by (a) relatively reacting one mole of a monofunctional, active-hydrogen-containing compound having at least 10 carbon atoms with between 20 and 400 moles of one or more alkylene oxides and (b) thereafter reacting the product of step (a) with a diepoxide in an amount such that the molar ratio of diepoxide to hydroxyl groups in the product of step (a) is between 0.2:1 and 5:1.

The present invention solves the problem defined above by employing a thickening agent of the type defined in US 3538033 in the applications described above, together with the formulation technology which is detailed below.

Considering the water component of the composition first, it is preferred that this comprises between 36 and 95% of the functional fluid most preferably between 45 and 80%.

As regards the glycol, this can be in principle any glycol which is miscible with water and includes monoethylene glycol and monopropylene glycol and low molecular weight oligomers thereof (ie having up to 6 ethylene and/or propylene glycol units). Preferably the glycol is selected from monoethylene glycol, diethylene glycol and triethylene glycol. It is preferred that the glycol comprises between 20 and 60% of the functional fluid.

The first stage of preparing the thickening agent involves reacting the monofunctional active hydrogen containing compound with one or more alkylene oxides. By the term 'active-hydrogen-containing compound' is meant one which contains hydrogen measurable by the Zerewitinoff active hydrogen test. Such compounds include alcohols, phenols, thiois, fatty acids and amines. The preferred compounds are C₁₆ to C₂₀ monohydric alcohol or thiols, C₁₆ to C₂₀ alkyl phenols and C₁₆ to C₂₀ aliphatic amines.

The active hydrogen containing compound is alkoxylated with one or more alkylene oxides using either a base or a Lewis acid as a catalyst. Typically the alkylene oxide is one or more of ethylene oxide, propylene oxide or the isomers of butylene oxide. Suitably between 20 and 400 moles of the alkylene oxide are added to the active hydrogen containing compound of which 20 to 100 mole % (most preferably 65 to 85 mole %) is ethylene oxide and 0 to 80% (most preferably 15 to 35%) is propylene and/or butylene oxide.

In the second stage of manufacture the product of the first stage is reacted with a diepoxide. The diepoxide can in principle be any organic compound having two epoxide groupings. Suitable diepoxides are those having between 4 and 30 carbon atoms and include vinylcyclohexene diepoxide, bisphenol A/epichlorohydrin condensate and the like. It is preferred to use the diepoxide in amounts such that the molar ratio of epoxide groups to hydroxyl groups (in the product of stage 1) is in the range 0.2 to 1 to 5 to 1. The second stage of the process can also be catalysed by either a base or a Lewis acid.

It is preferred that the thickening agent comprises between 2 and 10% by weight of the functional fluid composition. It is also preferred that the thickener itself should have a neat viscosity in excess of 4000 cSt at 40°C.

Concerning the antiwear components, these are typically metal or amine salts of organo sulphur, phosphorus or boron derivatives, or carboxylic acids. Typically these include salts of C₁ to C₂₂ carboxylic acids, aliphatic or aromatic; sulphur acids such as aromatic sulphonic acids, phosphorus acids, for example acid phosphate esters and analogous sulphur compounds, eg thiophosphoric and dithiophosphoric acid. Many further antiwear agents are suitable, and known to the skilled man.

Inhibitors for corrosion of metals can be organic or inorganic, for example metal nitrites, hydroxyamines, neutralised fatty acid carboxylates, phosphates, sarcosines and succinimides etc. Most useful are amines such as alkanolamines, e.g. ethanolamine, diethanolamine and triethanolamine. Non-ferrous metal inhibitors include for example aromatic triazoles.

It is preferred to include in the formulation 0.5 to 15% of a surfactant as a co-thickening agent, which may be non-ionic, cationic, anionic or amphoteric. Examples of suitable surfactants include linear alcohol alkoxylates, nonylphenol ethoxylates. fatty acid soaps, amine oxides etc. Most preferred are linear secondary alcohol alkoxylates, eg those commercially available from BP Chemicals under the registered trade mark Softanol. The surfactants behave synergistically with the associative thickener, such that a given viscosity can be achieved with a lower total thickener content of the blend compared to use of the associative thickener alone.

In addition to the above the functional fluid composition may also contain optional components such as extreme pressure additives, antifoams, antimicrobials and the like which are well known to the skilled man. It is also possible to add further known thickening agents and co-thickening agents if desired.

The functional fluid compositions of the present invention may be prepared by mixing the four main components and any additional materials which are required in a vessel of suitable size.

In the preferred embodiments of the invention, that is those formulations containing 20 or more percent of glycol, it has been found that temporary shear stability is conferred to the fluids. This enhances the capability of the fluids to provide hydrodynamic lubrication under high shearing conditions. The presence of the 20 or more percent glycol, and of the surfactant cothickener also improves the apparent viscosity index of the fluids when compared against fluids containing no glycol or surfactant.

In those embodiments of the invention containing less than 20 percent glycol, the problem of temporary shear is also addressed, by use of associative thickeners of the present invention with high inherent polymer viscosity (eg greater than 20,000 cSt at 40°C). In high shear environments, thickening achieved by association is lost when the fluids shear temporarily. However, the viscosity of the fluid is maintained at an intermediate level by the normal thickening of a high viscosity polymer, typically to a level of 10-20 cSt at 50°C. This limits the loss of pump efficiency, and ensures that hydrodynamic lubricity is retained. This approach also enhances the characteristics of the fluid concerning viscosity change on water loss and viscosity index.

The functional fluid compositions of the present invention are particularily useful as hydraulic fluids in piston, gear or vane hydraulic pumps, motors and general hydraulic systems, eg hydraulic rams, robots and the like.

The invention is now illustrated by the following examples:

### Example 1

A commercial sample of oleyl/cetyl alcohol (85/15) was catalysed with potassium hydroxide (0.3% by weight on the target alkoxylate), dried, and reacted with a 70/30 (weight/weight) mixture of ethylene oxide and propylene oxide at 115-125°C to produce an alkoxylate having an experimentally determined molecular weight of 6000 (by hydroxyl determination).

500 grams of the above un-neutralised alkoxylate was reacted at 130°C with 15.9 grams bisphenol A/epichlorohydrin condensate (Epikote 828 - ex Shell) for three hours. The residual catalyst was removed by treatment with magnesium silicate to leave an associative thickener with a neat viscosity of 5000 cSt @ 40°C. A 10% aqueous solution viscosity was determined as 193 cSt @ 40°C.

### Example 2

500 grams of the above-mentioned un-neutralised alkoxylate from example 1 was reacted at 130°C with 31.8 grams of bisphenol A/epichlorohydrin condensate for 3 hours, the catalyst was removed with magnesium silicate treatment, to leave an associative thickener with a neat viscosity of 17,300 cSt @ 40°C. A 10% aqueous solution viscosity was determined as 2100 cSt @ 40°C.

### Example 3

A commercial sample of oleyl/cetyl alcohol (85/15) was reacted in the manner described in example 1 with an 80/20 mixture of ethylene oxide and propylene oxide to produce an alkoxylate having a molecular weight of 6000.

300 grams of the above-mentioned un-neutralised polyalkylene glycol was reacted with 14.0 grams of vinylcyclohexene diepoxide for three hours at 140-150°C. The resulting associative thickener had a neat viscosity of 4,900 cSt @ 40°C and a 10% aqueous solution viscosity of 1427 cSt @ 40°C.

### Example 4

A commercial sample of oleyl/cetyl alcohol (85/15) was reacted in the manner described in example 1 with an 75/25 mixture of ethylene oxide and propylene oxide to produce an intermediate having a molecular weight of 2950, then with further ethylene oxide to produce an alkoxylate having a molecular weight of 3100.

2000 grams of the above mentioned un-neutralised polyalkylene glycol was reacted with 175 grams of vinylcyclohexene diepoxide at 140-150°C for 6 hours to yield an associative thickener with a 10% aqueous solution viscosity of 1742 cSt.

### Examples 5 - 8

Dodecan-1-ol, Tetradecan-1-ol, Hexadeca-1-ol and Octadecan-1-ol were reacted under base catalysis with 80/20 blends of ethylene oxide/propylene oxide to produce alkoxylates having molecular weights of 6000. 200 grams of each alkoxylate was reacted with 9.4 grams of vinylcyclohexene diepoxide in the manner described for example 3 to yield four associative thickeners. The products were used to provide a comparison of solution viscosity versus hydrophobe chain length.

### Example 9

The thickener (8%) from example 1 was formulated into a hydraulic fluid of 46 cSt at 40°C containing water (36%), diethylene glycol (50%), a fatty acid and morpholine. This was subjected to a four ball test (IP239) at 40 kg for 1h, and gave a wear scar of 0.56 mm, a result similar to that of a similarly formulated hydraulic fluid using 15% of a conventional polyglycol thickener.

The same thickener at a level of 7% in a high water based fluid of 46 cSt at 40°C was subjected to 50 passes in a Kurt Orban shear stability tester (IP294) and suffered no permanent loss of solution viscosity.

### Example 10

The thickener from example 4 was formulated at a level of 8% into a hydraulic fluid containing 30% diethylene glycol and 58% water, the balance being an antiwear and anticorrosion package. The said hydraulic fluid was circulated over 24 hours in a 7 kW Vickers PFB-5 axial piston pump at 50°C and 170 bar. The flow rate, which can be directly related to the fluid viscosity, was monitored to indicate viscosity in the high shear regions of the pump. The said hydraulic fluid was compared to a similar hydraulic fluid containing only 10% diethylene glycol and 80% water, and with a further hydraulic fluid, based on a commercially available, low-viscosity, associative thickener, a fatty alcohol ethoxylate capped with an olefin epoxide, and containing no diethylene glycol.

### Example 11

The thickener from example 1 (6.2%) and a 5 mole ethoxylate of a linear secondary C-12/14 alcohol (1.55%) (Softanol 50 - ex BP Chemicals) were blended with diethylene glycol (40%) and water (50%), the balance consisting of functional antiwear, anticorrosion and antifoam agents (2.25%) to give a hydraulic fluid of 45.5 cSt @ 40°C. The following data were determined.
Four ball wear scar, mm (1h, 40kg, IP239): 0.61
Shear Stability (IP294), % viscosity change: -7

### Example 12

The associative thickener from example 3 (3.6%) and a 5-mole ethoxylate of a linear secondary C-12/14 alcohol (0.9%) were blended with diethylene glycol (20%) and water (73.4%), the balance being additives (2%), to give a hydraulic fluid of 49.3 cSt @ 40°C. The following data were determined.
Four ball wear scar, mm (1h, 40kg, IP239): 0.62
Shear Stability (IP294), % viscosity change: +5

### Example 13

The associative thickener from example 3 (5.4%) and a 12 mole ethoxylate of a linear secondary C-12/14 alcohol (3.6%) (Softanol 120 - ex BP Chemicals) were blended with diethylene glycol (39%) and water (50%), the balance consisting of antiwear anticorrosion, antifoam additives (2%), to give a hydraulic fluid of 46.8 cSt @ 40°C. The following data were determined.
Four ball wear scar, mm (1h, 40kg, IP239): 0.61
Shear Stability (IP294), % viscosity change: +2.9

### Example 14

The thickener from example 2 (5.0%) and a 12 mole ethoxylate of a linear, secondary, C12/14 alcohol (1.25%) were blended with diethylene glycol (20%) and water (70%), the balance consisting of antiwear, anticorrosion and antifoam agents (3.75%) to give a hydraulic fluid of 46.1 cSt @ 40°C. The following data were determined.
Four ball wear scar, mm (1h, 40kg, IP239): 0.68

### Example 15

To demonstrate the effect of diethylene glycol on apparent viscosity index two ISO 68 fluids were prepared from the thickener from example 3. Fluid 1 containing 6.0 percent of thickener, 30 percent of diethylene glycol and 64 percent of water. Fluid 2 containing 5.0 percent thickener and 95 percent water. The combined effect of the presence of diethylene glycol and the slightly increased thickener requirement in fluid 1 results in a significantly lower viscosity fluid at 20°C than that observed for fluid 2, demonstrating that the apparent viscosity index of fluid 1 is higher than that of fluid 2.

### Example 16

To demonstrate the effect of co-thickeners on apparent viscosity index, two fluids of 550 cSt @ 40°C were prepared as follows: Fluid 1 contained 6.0 percent of thickener from example 2, 4.0 percent of a 12 mole ethoxylate of a C-12/14 linear secondary alcohol, 10 percent diethylene glycol and 80 percent water. Fluid 2 contained 10.0 percent thickener from example 2, 10 percent diethylene glycol and 80 percent water. The presence of surfactant in fluid 1 and reduced thickener requirement results in a significantly lower viscosity fluid at 20°C than observed for fluid 2, demonstrating that the apparent viscosity index of fluid 1 is higher than that for fluid 2.

## Claims

1. A functional fluid composition for use as a hydraulic fluid, lubricant, cutting fluid or drilling fluid which comprises
(a) from 20 to 98% by weight water
(b) a finite amount of up to 79.5% by weight of glycol and
(c) from 0.5 to 25% by weight of a thickening agent prepared by (i) relatively reacting one mole of a monofunctional active-hydrogen-containing compound having at least 10 carbon atoms with between 20 and 400 moles of one or more alkylene oxides and (ii) thereafter reacting the product of step (i) with a diepoxide in an amount such that the molar ratio of diepoxide to hydroxyl groups in the product of step (i) is between 0.2:1 and 5:1.

2. A functional fluid composition as claimed in claim 1 further comprising functional components for preventing wear and corrosion.

3. A functional fluid composition as claimed in claim 1 comprising from 35 to 95% by weight water.

4. A functional fluid composition as claimed in claim 1 comprising from 20 to 60% by weight glycol.

5. A functional fluid composition as claimed in claim 1 comprising 2 to 10% by weight of the thickening agent.

6. A functional fluid as claimed in claim 1 or claim 4 further comprising 0.5 to 15% by weight of a non-ionic, cationic, anionic or amphoteric surfactant.

7. A functional fluid composition as claimed in claim 1 comprising a finite amount of up to 20% by weight glycol and 0.5 to 25% by weight of a thickening agent having a neat viscosity greater than 20,000 cSt at 40°C.

8. A functional fluid as claimed in claim 1 wherein component (c) is prepared by reacting one mole of a monofunctional active-hydrogen-containing compound having at least 10 carbon atoms with between 20 and 400 moles of a mixture of ethylene and propylene oxide to form an intermediate and thereafter capping the intermediate with up to 4 moles of ethylene oxide and (ii) thereafter reacting the product of step (i) with a diepoxide in an amount such that the molar ratio of diepoxide to hydroxyl groups in the product of step (i) is between 0.2:1 and 5:1.

9. A process for preparing a functional fluid as defined in claim 1 which comprises mixing the required amounts of water, glycol and thickening agent.

10. A process as claimed in claim 9 in which functional components for preventing wear and corrosion are added during mixing.

## Patentansprüche

1. Funktionsfluid-Zusammensetzung für die Verwendung als hydraulisches Fluid, Schmierstoff, Schneidefluid oder Bohrfluid umfassend:
(a) von 20 bis 98 Gew.-% Wasser
(b) eine bestimmte Menge von bis zu 79,5 Gew.-% Glykol und
(c) von 0,5 bis 25 Gew.-% eines Andickungsagens, hergestellt durch (i) jeweils die Umsetzung eines Mols einer monofunktionellen aktiven Wasserstoff enthaltenden Verbindung, die wenigstens 10 Kohlenstoffatome besitzt mit zwischen 20 und 400 Mol eines oder mehrerer Alkylenoxide und (ii) danach Umsetzung des Produkts von Stufe (i) mit einem Diepoxid in einer Menge, so daß das molare Verhältnis von Diepoxid zu Hydroxylgruppen in dem Produkt von Stufe (i) zwischen 0,2:1 und 5:1 liegt.

2. Funktionsfluid-Zusammensetzung nach Anspruch 1, weiterhin beinhaltend Funktionskomponenten zur Verhinderung von Verschleiß und Korrosion.

3. Funktionsfluid-Zusammensetzung nach Anspruch 1, beinhaltend von 35 bis 95 Gew.-% Wasser.

4. Funktionsfluid -Zusammensetzung nach Anspruch 1, beinhaltend von 20 bis 60 Gew.-% Glykol.

5. Funktionsfluid-Zusammensetzung nach Anspruch 1, beinhaltend 2 bis 10 Gew.-% des Andickungsmittels.

6. Funktionsfluid-Zusammensetzung nach Anspruch 1 oder Anspruch 4, weiterhin beinhaltend 0,5 bis 15 Gew.-% eines nichtionischen, kationischen, anionischen oder amphoteren oberflächenaktiven Stoffes.

7. Funktionsfluid-Zusammensetzung nach Anspruch 1, beinhaltend eine bestimmte Menge von bis zu 20 Gew.-% Glykol und 0,5 bis 25 Gew.-% eines Andickungsagens mit einer reinen Viskosität größer als 20 000 cSt bei 40°C.

8. Funktionsfluid nach Anspruch 1, worin Komponente (c) hergestellt ist durch Umsetzen eines Mols einer monofunktionellen aktiven Wasserstoff enthaltenden Verbindung, die wenigstens 10 Kohlenstoffatome besitzt mit zwischen 20 und 400 mol einer Mischung aus Ethylen- und Propylenoxid, um ein Zwischenprodukt zu bilden und danach das Zwischenprodukt mit bis zu 4 Mol von Ethylenoxid zu überdecken und (ii) danach das Produkt aus Stufe (i) mit einem Diepoxid in einer solchen Menge, daß das molare Verhältnis von Diepoxid zu Hydroxylgruppen in dem Produkt aus der Stufe (i) zwischen 0,2:1 und 5:1 liegt, zur Reaktion bringen.

9. Verfahren zur Herstellung eines Funktionsfluides wie in Anspruch 1 definiert, beinhaltend das Mischen der benötigten Mengen von Wasser, Glykol und Andickungsmittel .

10. Verfahren nach in Anspruch 9, in welchem Funktionskomponenten zur Verhinderung von Verschleiß und Korrosion während des Mischens hinzugefügt werden.

## Revendications

1. Composition de fluide fonctionnel destinée à être utilisée comme fluide hydraulique, lubrifiant, fluide de coupe ou fluide de forage, qui comprend
(a) 20 à 98 % en poids d'eau
(b) une quantité finie allant jusqu'à 79,5 % en poids de glycol et
(c) 0,5 à 25 % en poids d'un agent épaississant préparé par (i) réaction relative d'une mole d'un composé monofonctionnel contenant de l'hydrogène actif ayant au moins 10 atomes de carbone avec entre 20 et 400 moles d'un ou plusieurs oxydes d'alkylènes, puis (ii) réaction du produit de l'étape (i) avec un diépoxyde en une quantité telle que le rapport molaire des groupes diépoxyde aux groupes hydroxyle dans le produit de l'étape (i) ait une valeur comprise entre 0,2:1 et 5:1.

2. Composition de fluide fonctionnel suivant la revendication 1, comprenant en outre des composants fonctionnels servant à empêcher l'usure et la corrosion.

3. Composition de fluide fonctionnel suivant la revendication 1, comprenant 35 à 95 % en poids d'eau.

4. Composition de fluide fonctionnel suivant la revendication 1, comprenant 20 à 60 % en poids de glycol.

5. Composition de fluide fonctionnel suivant la revendication 1, comprenant 2 à 10 % en poids de l'agent épaississant.

6. Composition de fluide fonctionnel suivant la revendication 1 ou la revendication 4, comprenant en outre 0,5 à 15 % en poids d'un surfactant non ionique, cationique, anionique ou amphotère.

7. Composition de fluide fonctionnel suivant la revendication 1, comprenant une quantité finie allant jusqu'à 20 % en poids de glycol et 0,5 à 25 % en poids d'un agent épaississant ayant une viscosité à l'état non dilué supérieure à 20 000 cSt à 40°C.

8. Composition de fluide fonctionnel suivant la revendication 1, dans lequel on prépare le composant (c) (i) en faisant réagir une mole d'un composé monofonctionnel contenant de l'hydrogène actif ayant au moins 10 atomes de carbone avec entre 20 et 400 moles d'un mélange d'oxyde d'éthylène et d'oxyde de propylène pour former un produit intermédiaire et en coiffant ensuite le produit intermédiaire avec jusqu'à 4 moles d'oxyde d'éthylène, puis (ii) en faisant réagir le produit de l'étape (i) avec un diépoxyde en une quantité telle que le rapport molaire des groupes diépoxyde aux groupes hydroxyle dans le produit de l'étape (i) se situe entre 0,2:1 et 5:1.

9. Procédé de préparation d'une composition de fluide fonctionnel tel que défini dans la revendication 1, qui comprend le mélange des quantités désirées d'eau, de glycol et d'agent épaississant.

10. Procédé suivant la revendication 9, dans lequel des composants fonctionnels servant à empêcher l'usure et la corrosion sont ajoutés pendant l'opération de mélange.
